

UNITED STATES PATENT OFFICE

2,396,396

## **PRODUCTION OF COLORED PHOTOGRAPHIC IMAGES**

Douglas William Stammers, Blackley, Manchester, England, assignor to Imperial Chemical Industries Limited, a corporation of Great Britain

**No Drawing. Application November 15, 1943, Serial No. 510,373. In Great Britain November 25, 1942**

4 Claims. (Cl. 95—6)

This invention relates to the production of colored photographic images.

It is known that when a photographic silver halide emulsion is developed by treatment with an aromatic amino developing agent, for example, an asymmetric dialkyl p-phenylenediamine, there is formed an image of metallic silver. It is also known that when there is present also in the developing solution or in the silver halide emulsion a suitable substance, known as a color-former, which will react with the oxidation product of the developer to produce a dyestuff there is also formed simultaneously a colored photographic image. The colored image may be revealed by removal of the silver image by treatment with a suitable bleaching agent, for example with that known as Farmer's reducer.

According to the present invention I produce a photographic dyestuff image in a photographic element either by developing a reducible silver salt contained in the element with an aromatic amino developing agent, as defined hereinafter, in the presence of a color former which is a 2:4-diarylpyrrole of the formula—



where  $R^1$  and  $R^{11}$  stand for aryl radicals for example of the benzene or naphthalene series, substituted or not, the same or different, and where  $R^{111}$  stands for hydrogen or for a non-reactive substituent, for example an aryl-, alkyl-, alkylamino-, benzylideneamino- or acylamino- radical, or by treating a photographic element containing such color former with an oxidation product of such a developing agent or with a p-nitrosodialkylaniline or with a diazonium salt.

The aromatic amino developing agents used are those which are capable of developing silver halide photographic emulsions and which are o- or p-phenylene diamines or derivatives thereof containing at least one unsubstituted amino-group, or o- or p-amino phenols or derivatives thereof containing an unsubstituted amino group. Examples of such developing agents which may be used include p-aminodimethylaniline, p-aminodiethylaniline, p-amino di-n-butyylaniline, p-methylaminoaniline, p-ethylaminoaniline, chloro-p-phenylenediamine, 1:2:5-toluylenediamine, 2-amino-5-diethylaminotoluene, N-p-aminophenylpiperidine, N-methyl-N- $\beta$ -hydroxyethyl-p-phenylenediamine, N-n-butyl-N- $\beta$ -hydroxyethyl-p-phenylenediamine,  $\beta$ - $\gamma$ -dihydroxy-

propyl-p-phenylenediamine and N:N-diethyl-o-phenylenediamine.

The 2:4-diarylpyrroles which may be used as color formers according to the invention include, for example, 2:4-diphenylpyrrole, 2-(p-methoxy-phenyl)-4-phenylpyrrole, 2-(m-hydroxyphenyl)-4-phenylpyrrole, 2-(o-chlorophenyl)-4-phenylpyrrole, 2-(p-acetylaminophenyl)-4-phenylpyrrole, 2- $\alpha$ -naphthyl-4-phenylpyrrole, 2-phenyl-4- $\beta$ -naphthylpyrrole, 2:3:4-triphenylpyrrole, 3-benzoylamino-2:4-diphenylpyrrole, 3-acetylamo-2:4-diphenylpyrrole and 3-benzoylamino-2:4-di-p-tolylpyrrole. The sulphonic acid derivatives of the 2:4-diaryl pyrroles, for example of those listed above, and their salts, may also be used.

The 2:4-diarylpurroles which are used as color formers may be made, for example, by the processes described in the specifications of applications Nos. 16,277/41 and 3,583/42, now British Patent No. 556,152, and in the processes involving

- 20 Patent No. 556,156 and in the corresponding United States applications Serial No. 457,229, filed September 3, 1942, and Serial No. 475,434, filed February 10, 1943. Those 2:4-diarylpyrroles which bear in the 3-position an amino or substituted amino group may be made as is described, for example, in the case of 3-benzoylamino-2:4-diphenylpyrrole, by Gabriel, in Berichte der deutschen chemischen Gesellschaft, 41, 1138. The sulphonic acid derivatives of the 2:4-diarylpyrroles may be made, for example, as is described in the specification of application No. 9,689/42 and corresponding United States application Serial No. 482,479, filed April 9, 1943.

As said the photographic dyestuff image may be produced by developing a reducible silver salt image with an aromatic amino developing agent in the presence of the color formers of the invention.

40 The color formers may be present in the developing solution or they may be incorporated in the photographic elements. Those sulphonated derivatives of the aforesaid 2:4-diarylpyrroles and their salts which are water-soluble are especially suitable for use in the developing solution. Those 45 color formers which are not sulphonated acid derivatives are frequently but sparingly soluble in water. Nevertheless, especially when they contain other solubilising groups, for example phenol groups, they may frequently be incorporated in 50 developing solutions by the use of suitable proportions of an organic solvent which is miscible with water, for example of ethanol. However, they are advantageously incorporated in the photographic emulsions and many of them, being 55 colorless or nearly so, are highly suitable for this

purpose. Being also sparingly soluble in water they have little tendency to diffuse from the film into the processing solutions. The color formers of the invention may be incorporated in the photographic emulsions by any of the well known methods, for example by the processes described in British specifications Nos. 540,368 and 541,558.

The images obtained using the color formers of the invention are of bright reddish blue to blue-green shades. These shades are of high intensity and, furthermore, they are of high intensity when, as is desirably the case, photographic developing solutions are used which contain an alkali metal sulphite.

As is known, many of the blue-green images obtained from known color formers, which should, ideally, transmit all light of 400-500 m $\mu$ , wave length do in fact absorb appreciably in this region. Thus for example in making copies from colored originals by methods in which no color correction by masking is introduced, there is thereby introduced a shift of hue whereby in effect there is superimposed yellow over the blue areas of the copy. I have found that certain of the color formers of this invention, particularly those in which the aryl groups of the 2:4-diaryl-pyrroles are substituted by chlorine atoms, give rise to dye images which show an improved transmission in the 400-500 m $\mu$ , i. e., blue, region.

As illustrated in the examples which follow the photographic images are produced in photographic elements containing a reducible silver salt image by development with an aromatic amino developing agent. But, as already stated, alternative methods may be used. Thus an element containing the color former may be treated with the oxidation product of an aromatic amino developing agent. For example the color former may be incorporated in bichromate-sensitised colloid layers, for example gelatin, gum arabic or albumen, the layers exposed, the unexposed colloid removed, for example by treatment with hot water, and the color developed in the exposed portions by treatment with a p-nitrosodiamylaniline or a derivative thereof.

Furthermore, photographic elements containing the color formers of the invention may be treated with diazonium salts to form azo dyes. Thus when treated with benzene diazonium chloride the color formers of this invention yield yellow or red dyes which may readily be differentially bleached to form dye images, for example by the processes of British specifications Nos. 133,034 and 496,558.

The invention is illustrated but not limited by the following examples:

#### Example 1

To 1000 cc. of a developer having the following composition:

|                                                 |       |       |
|-------------------------------------------------|-------|-------|
| Sodium sulphite (cryst.)                        | grams | 15.0  |
| 2-amino - 5 - diethylaminotoluene hydrochloride | grams | 3.0   |
| Sodium carbonate (anhyd.)                       | do    | 40.0  |
| Potassium bromide                               | do    | 0.5   |
| Water to                                        | ccs.  | 1,000 |

there is added 100 ccs. of a solution of 1.0 gram of 2-phenyl-4-(m-hydroxylphenyl)pyrrole and 2.9 grams of sodium hydroxide in 100 ccs. of a mixture of equal weights of water and ethanol.

When a photographic element containing reducible silver salts is developed in this solution a bright greenish-blue dye image is produced together with metallic silver. The silver may be

removed from the element by successive bathing in a 4% aqueous solution of potassium ferricyanide and in a 25% aqueous solution of sodium thiosulphate.

5

#### Example 2

1.0 gram of the sodium salt of 2-phenyl-4-(o-chlorophenyl)pyrrole monosulphonic acid is dissolved in 100 ccs. of hot water and the solution is added to 1000 ccs. of the developing solution used in Example 1.

When a photographic element containing reducible silver salts is developed in this solution a clear greenish-blue dye image is produced together with metallic silver.

15

#### Example 3

1.0 gram of the sodium salt of 2-phenyl-4-(p-methoxyphenyl)pyrrole monosulphonic acid is dissolved in 100 cc. of hot water and the solution is added to 1000 cc. of the developing solution used in Example 1.

When a photographic element containing reducible silver salts is developed in this solution a blue dye image is obtained. The silver may be removed without detriment to the dye image by alternate treatment with potassium ferricyanide and sodium thiosulphate as is described in Example 1.

20

#### Example 4

1.0 gram of the ammonium salt of 2:4-di-phenylpyrrole monosulphonic acid is dissolved in a mixture of 50 ccs. of water and 50 ccs. of acetone. A further 50 ccs. of acetone are added to the solution and the resulting mixture is added to 1000 ccs. of a developer of the following composition:

|                                                 |       |       |
|-------------------------------------------------|-------|-------|
| Crystalline sodium sulphite                     | grams | 15.0  |
| Asymmetric diethyl p-phenyl-enediamine sulphate | grams | 3.0   |
| Anhydrous sodium carbonate                      | do    | 40.0  |
| Potassium bromide                               | do    | 0.5   |
| Water to                                        | ccs.  | 1,000 |

30

A photographic element containing a developable silver halide image is treated with the above solution and a bright blue dye image is obtained together with the silver image.

35

#### Example 5

To 1000 ccs. of the developing solution used in Example 1 there is added 100 ccs. of acetone and the resulting mixture is employed as a developer for a photographic element containing a reducible silver salt and also containing 2-phenyl-4-(2-chlorophenyl)pyrrole in the form of a fine uniform dispersion. A bright greenish-blue dye image is obtained along with the silver image.

40

Photographic elements containing other color formers are developed in the developing solution used in Example 5. The color of the dye image obtained is shown in the table below:

| Ex-<br>ample<br>No. | Color Former                            | Color of image |
|---------------------|-----------------------------------------|----------------|
| 6                   | 3-benzoylamino-2:4-diphenylpyrrole      | Blue.          |
| 7                   | 2-phenyl-4-(p-methoxyphenyl)pyrrole     | Do.            |
| 8                   | 2:4-diphenylpyrrole                     | Do.            |
| 9                   | 2-phenyl-4-(p-bromophenyl)pyrrole       | Do.            |
| 10                  | 2-phenyl-4-( $\alpha$ -naphthyl)pyrrole | Greenish-blue. |

I claim:

1. A process for the production of a photographic dyestuff image which comprises developing a photographic element containing a reduc-

45

ible silver salt image with an aromatic primary amino color developing agent in the presence of a substituted 2:4-diarylpyrrole of the formula



where  $\text{R}^{\text{I}}$  and  $\text{R}^{\text{II}}$  stand for aryl radicals and  $\text{R}^{\text{III}}$  stands for a member of the group consisting of hydrogen, aryl, alkyl, alkylamino, benzylidene-amino, and acylamino radicals.

2. A photographic element bearing an emulsion layer containing a light-sensitive material and a color former comprising a 2:4-diarylpyrrole of the formula



where  $\text{R}^{\text{I}}$  and  $\text{R}^{\text{II}}$  stand for aryl radicals and  $\text{R}^{\text{III}}$  stands for a member of the group consisting of hydrogen, aryl, alkyl, alkylamino, benzylidene-amino, and acylamino radicals.

3. A photographic element bearing a light-sen-

sitive silver halide emulsion layer containing a color former comprising a substituted 2:4-diarylpyrrole of the formula

5



where  $\text{R}^{\text{I}}$  and  $\text{R}^{\text{II}}$  stand for aryl radicals and  $\text{R}^{\text{III}}$  stands for a member of the group consisting of hydrogen, aryl, alkyl, alkylamino, benzylidene-amino, and acylamino radicals.

4. A photographic developing solution containing an aromatic primary amino color developing agent and a color former comprising a substituted 2:4-diarylpyrrole of the formula



20

where  $\text{R}^{\text{I}}$  and  $\text{R}^{\text{II}}$  stand for aryl radicals and  $\text{R}^{\text{III}}$  stands for a member of the group consisting of hydrogen, aryl, alkyl, alkylamino, benzylidene-amino, and acylamino radicals.

25

DOUGLAS WILLIAM STAMMERS.